

## UNITED STATES PATENT OFFICE

2,404,769

DIRECT DYE PLANOGRAPHIC PRINTING  
COMPOSITIONSChester A. Amick, Bound Brook, N. J., assignor to  
American Cyanamid Company, Bound Brook,  
N. J., a corporation of MaineNo Drawing. Application December 23, 1944,  
Serial No. 569,624

20 Claims. (Cl. 8—62)

1

This invention relates to putty compositions suitable for planographic printing on cellulosic material and leather employing dyes which are capable of being directly affixed to cellulosic material without mordanting.

In the past the printing of cellulosic material has been accomplished almost exclusively by use of the intaglio method. In this method a relatively free flowing printing paste containing the color to be printed is applied to an engraved printing roll, usually copper, for example by means of a furnisher roller, the excess paste scraped off the roller so that paste remains only in the depressions, and the roller applied to the fabric in a printing machine. This procedure, while satisfactory for many types of designs, has a number of disadvantages. In the first place, it is not possible to produce designs with extremely fine, close fitting, interwoven, multi-colored lines without a certain amount of running or smudging of the lines, because it is necessary to have a rather free flowing printing paste or otherwise it will not print satisfactorily. Multi-color printing is also a very serious problem because each color requires a separate roll and a sharp print requires accurate alignment and synchronism of the different printing rolls. When a great number of colors are to be printed a further disadvantage is the large amount of capital which has to be tied up in engraved rollers.

Planographic printing in which the surface is contacted with a solid putty or block of color and a portion of the color is transferred to form a print presents many operating advantages. This method of printing has not been applied to cellulosic fibers because when it was attempted to prepare direct dye compositions in the form of putties they showed a short softening range and in many cases were friable. The resulting prints showed specks and other unevenness and were not satisfactory. When it is attempted to use large amounts of glycerin or similar hygroscopic agents the product is still not satisfactory and does not keep in humid atmospheres which makes it impossible to use in commercial printing plants.

According to the present invention I have found that when putties are prepared containing dyes capable of being directly affixed to cellulosic material without mordanting, using the customary carbohydrate gum such as dextrin, products having a long softening range can be obtained if there is present an amide of carbonic,

2

thiocarbonic or cyanuric acids. The common amides are urea, thiourea and melamine, and in the case of urea and thiourea at least the amide is also an excellent fixing agent, thus performing both functions. While urea and thiourea are fixing agents, they are in no sense mordants, that is to say, they do not react with the dyestuff to form insoluble lakes. It is not desired to limit the present invention to a particular theory of action, but it seems reasonably certain that there is some chemical reaction or combination between the amide and carbohydrate. In the case of urea and thiourea, products having many of the properties of thermoplastic synthetic resins are obtained, the urea or thiourea appearing to react with the dextrin. In the case of melamine this resin formation is not apparent, although there may well be some reaction because melamine does not enhance the printing characteristics of the putty and increases the softening range of the putty.

The various amides are not all equally effective. Urea is the best. Thiourea gives almost as good results as urea but melamine, while permitting the production of useful prints, is not as effective as either urea or thiourea.

While the presence of the amide is the principal feature of the present invention and permits the production of useful printing putties with direct colors, for best results I find that certain other constituents are desirable, although not essential, for obtaining usable prints. Thus, I find that the incorporation in the putty of a waxy material, particularly a glyceryl monoster of a higher fatty acid, controls the plasticity of the putty, aids in giving the maximum softening range and also appears to enhance the transfer of the color in planographic printing, and in a more specific aspect of the invention the presence of such a waxy material is included.

Another feature, advantageous in producing prints of maximum quality, is the incorporation in the putty of a soap such as a low titre olive oil soap. The soap appears to improve the sharpness and strength of the print, but is not as important a feature as the incorporation of the waxy material.

While the present invention is useful with a wide variety of carbohydrate gums best results are obtained when the gums are more highly dextrinized than is common practice in ordinary printing pastes. Usually in such cases natural gums or a rather heavy bodied, not extensively dextrinized carbohydrate is employed, such as a

white dextrin of the British gum type. Experience with ordinary printing paste would lead one to expect that these materials would also give better bodied putties for planographic printing. I have found, however, that the contrary is the case when dealing with putties containing direct dyes suitable for planographic printing, the best putties being obtained when highly dextrinized materials such as yellow corn dextrin are used. This constitutes a feature of the preferred embodiment of the present invention and is of importance where results of the highest quality are required, although entirely satisfactory prints can be obtained with less highly dextrinized materials.

It is also desirable to incorporate in the putties a small amount of a wetting agent for which esters of sulfosuccinic acid have proven to be very useful and also a small amount of trisodium phosphate appears to improve the consistency of the putties.

Another ingredient which may be added and which is useful in producing the best results is bentonite, preferably in a somewhat hydrated or gelatinous form, and this is a further feature of the preferred embodiment of the invention.

While the softening ranges of the putties produced according to the present invention will vary, in general they display plasticity throughout a range running from about 37-40° F. up to 113° F., or even somewhat higher. This should be contrasted with putties prepared without the amides which show excessive hardness and friability at temperatures around 37° F. and are too soft to be coherent in the printing operation above 100° F.

While the proportions of carbohydrate gum, such as dextrin, amide and other constituents, are not critical, nevertheless there are certain ranges within which they must be kept in order to give putties which are satisfactory in their softening range and printing characteristics. Thus the putties may contain carbohydrate gum, such as dextrin, in amounts from 45 to 60% of the total weight. The amide may be used in amounts from 6 to 25% and the water content in general should be kept within the range of 5 to 15%. The optimum results will vary somewhat with the particular members chosen. For example, when a relatively large amount of urea is used with the dextrin somewhat less water should be employed in order to prevent formation of putties which have too low a softening point.

It is an advantage of the present invention that the putties have a long softening range which permits printing operations at elevated temperatures. The use of elevated temperatures in many cases presents advantages as the printing is accelerated and penetration of the fiber is improved. The long softening ranges of the putties of the present invention permit operating at moderately elevated temperatures and realizing the advantages which result from such operation.

The reference to cellulosic material in the present invention is not intended to be limited to natural cellulose fibers themselves. On the contrary, it includes not only natural cellulose fibers such as cotton, linen, and the like, but also regenerated cellulose such as viscose and other regenerated cellulosic rayons, and the like.

While the largest field of practical usefulness of the putties of the present invention lies in

the printing of ordinary cellulosic fibers such as cotton, regenerated cellulose and the like, it is an advantage that the putties are also useful in printing leather, which has hitherto raised a considerable problem with ordinary printing procedures.

Another field of usefulness of the present invention lies in the printing of so-called high wet-strength papers, that is to say, papers which have 10 urea formaldehyde, and particularly melamine formaldehyde resins, incorporated in or on the paper, as described in the article by Maxwell, Paper Trade Journal, vol. 116, No. 19, pages 39 to 42. Prints of excellent strength and sharpness 15 are obtainable in spite of the fact that this type of paper presents serious difficulties to ordinary printing processes, and in fact even planographic putties containing vat dyes, described in patent of Kienle, Amick and Kerns, No. 2,364,359, issued December 5, 1944, can only be used to give 20 pastel shades on wet strength paper. The putties of the present invention give sharp prints on this type of paper without bleeding and in any color strength desired.

25 The invention will be described in conjunction with the following specific examples, but it is not limited to the details therein set forth. The parts are by weight.

#### Example 1

30 120 parts of Calcomine Fast Scarlet 4BSY (C. I. 326) were pasted with 100 parts of ethyl ether of ethylene glycol and 600 parts of water. To this were added 480 parts of urea whereupon 35 the color appeared to go into solution. This color solution was then cold pasted with 1000 parts of yellow dextrin in a dough mixer until uniform. The steam valve was slightly open, the dextrin cooked at a temperature above 165° F. for 15 minutes. 200 parts olive oil soap, 40 parts 40 glyceryl mono stearate, 10 parts trisodium phosphate and 10 parts of isobutyl ester of sodium sulfosuccinic acid were added after having been previously pasted with 100 parts of boiling water 45 in a separate container. Evaporation of moisture from the dough mixer was continued under vacuum until a thin section, chilled by cooling on an ice cold tin, fractured when bent by hand or struck a blow with a blunt instrument. When 50 printed by the planographic method on a piece of pigmented rayon (i. e. on the moist material), this color was transferred uniformly, giving a bright, smooth, scarlet print. A satisfactory result was obtained when this color was printed 55 by the planographic method on a piece of cotton fabric.

#### Example 2

60 750 parts of the product prepared in the preceding example and 150 parts of a 7% bentonite gel containing 1% sodium carbonate were worked in a small dough mixer to which heat was applied externally from a Bunsen burner. The water was evaporated until the same test was obtained as in Example 1. This product gave good smooth prints when applied planographically to pigmented rayon and cotton. The addition of the bentonite reduced the tackiness of the solid product as compared to that obtained in Example 1.

#### Example 3

70 120 parts of Direct Sky Blue FF (C. I. 518) were pasted with 100 parts of ethyl ether of ethylene glycol and 600 parts of water. To this

## 5

were added 480 parts of urea whereupon the color appeared to go into solution. This color solution was then cold pasted with 1000 parts of yellow dextrin in a dough mixer until uniform. The steam valve was slightly open, the dextrin cooked at a temperature about 160° F. for 15 minutes. 200 parts of olive oil soap, 40 parts glyceryl mono stearate, 10 parts trisodium phosphate, and 10 parts of isobutyl ester of sodium sulfosuccinic acid were added after having been previously pasted with 100 parts of boiling water in a separate container. Evaporation of moisture from the dough mixer was continued under vacuum until a thin section, chilled by cooling on an ice cold tin, fractured when bent by hand or struck a blow with a blunt instrument. When printed by the planographic method on a piece of pigmented rayon, this color transferred uniformly giving a bright, smooth blue print.

## Example 4

Pieces of the products of Examples 1, 2, and 3 were formed into a composite printing block in the form of a design in the different colors. When printed by planographic methods on pigmented rayon a sharp print of the design in the different colors was obtained. No tendency toward running of the edges of the different colors in the designs was noted.

## Example 5

The procedure of Example 1 was followed except that the urea was replaced by thiourea. The colored product obtained gave bright prints and was entirely satisfactory. When thiourea and dextrin were added together without the other substituents a resin-like product was obtained, the elastic properties of which were only slightly inferior to the corresponding product with urea and dextrin.

## Example 6

The procedure of Example 1 was followed but the urea was replaced by the same amount of melamine. The product obtained gave satisfactory prints, but did not have quite the elasticity and softening range of the products using urea or thiourea.

## Example 7

120 parts of the dye having Color Index No. 666 are pasted with 100 parts of the ethyl ether of ethylene glycol and 600 parts of hot water, after which 480 parts of urea are added. 1,000 parts of corn dextrin, sold by Stein-Hall under the trade name 4-H, was then added to a small Werner-Pfleiderer steam heated laboratory vacuum dough mixer, the above color solution added and stirred until uniform. It was then heated to 150° F.

150 parts of an olive oil soap powder, 40 parts of glyceryl monostearate, 10 parts of sodium di-isobutyl sulfosuccinate, 10 parts of trisodium phosphate, and 100 parts of boiling water are pasted and then added to the color-dextrin composition in the mixer. The mix is then dried under five inches of vacuum at 80°-85° C. until a cold thin piece fractures when bent or struck a sharp blow with a hammer.

A piece of moist titanium-dioxide pigmented viscose-rayon is used to make planographic prints of the above composition. After drying, the printed pieces are lightly wrapped in a white 80 x 80 cotton percale and steamed for 10 and 45 minutes respectively in an open steamer, and

## 6

other pieces are steamed for 45 minutes in a cottage or pressure steamer at five pounds pressure. All these prints showed exceptional fastness for this color.

## Example 8

The preceding experiment is repeated exactly except 40 parts of di-ethylene glycol monolaurate are added. Planographic prints obtained from this color composition had even better color values than those obtained from the composition prepared in Example 7.

## Example 9

1,000 parts of the product sold by Stein-Hall as S-S Dextrine are pasted in a Werner-Pfleiderer mixer with 250 parts of water. When uniform, the dextrin paste is heated by admitting steam into the steam jacket. The heating and stirring are continued until the paste has hydrated. 40 parts of glyceryl monostearate, 160 parts of Lux soap sold by Lever Brothers, 10 parts of sodium di-isobutyl sulfosuccinate and 10 parts of trisodium phosphate are pasted with 100 parts of water. This composition is then added to the hot dextrin paste and stirring and heating continued. 120 parts of the dye having Color Index No. 382 are then pasted with 120 parts of the ethyl ether of ethylene glycol and 120 parts of water, after which the color mixture is added to the other ingredients in the mixer. Finally, 120 parts of urea crystals are added, after which, heating, mixing and evaporation of moisture is continued until a cooled thin section fractures when struck a blow with a hammer.

When this composition is printed on a piece of moist 80 x 80 cotton percale or titanium dioxide pigmented viscose rayon fabric or on absorbent paper, dried, then steamed for half an hour in an open steamer, a bright scarlet print of good fastness is obtained.

## Example 10

A composition is prepared as in the preceding example except the dye having Color Index No. 561 is used in place of the dye having Color Index No. 382.

## Example 11

A composition is prepared as in Example 9 except the dye having Color Index No. 698 is used in place of the dye having Color Index No. 382.

## Example 12

A composition is prepared as in Example 9 except the dye having Color Index No. 620 is used in place of the dye having Color Index No. 382.

## Example 13

A composition is prepared as in Example 9 except the dye having Color Index No. 1078 is used in place of the dye having Color Index No. 382.

## Example 14

A printing color block was prepared using the color compositions of the last five examples. A piece of moist titanium dioxide pigmented viscose rayon was printed with this composition. After printing, drying and steaming, a brightly colored fabric was obtained. A piece of wet strength paper prepared according to the description of the Maxwell article referred to above was moistened and printed with the printing color block. A bright colored print was obtained which was 75 resistant to running water, even when fairly hot.

A moist piece of transparent velvet, having a viscose rayon pile, was printed by the planographic process using this printing color block and after drying, steaming, and washing, an excellent transfer of color was obtained, resulting in a good bright print.

A piece of moist leather was printed on the printing color block. The color transferred and gave a well penetrated print without steaming.

A moist woolen pile fabric on a cellulosic back was printed with the printing color block. After steaming, an excellently printed pattern was obtained.

*Example 15*

A printing color block was prepared using the composition made in Examples 1, 3 and 7. This was used to print planographically a piece of titanium dioxide pigmented viscose rayon. After drying and steaming, the fabric was colored strongly and evenly.

While it is an advantage of the present invention that a large number of dyes capable of being directly affixed to cellulose without mordanting can be used, the dyes do not all behave exactly alike. Some of them give good color values simply by printing, drying, washing, and again drying. In the case of other dyes which are in the majority the color value and fastness properties are improved by steaming in a continuous steamer or in a pressure steamer at about five pounds pressure. In either case the steaming is usually continued for from 15 to 60 minutes. Where steaming is referred to in the examples, dyes are used which require steaming to bring out the best strength and fastness.

This application is in part a continuation of my copending application, Serial No. 475,049, filed February 6, 1943, which is in turn a continuation in part of my earlier application, Serial No. 364,531, filed November 6, 1940.

I claim:

1. A putty suitable for planographic printing comprising a color capable of being directly fixed on cellulose without mordanting, a carbohydrate gum as the essential bodying ingredient and an amide of an acid included in the group consisting of carbonic acid, thiocarbonic acid and cyanuric acid, all of the ionizable hydrogen atoms of the acid being amidified and the amide having at least one free reactive hydrogen atom and being present in the form of a reaction product with the carbohydrate gum, the putty being hard at room temperature, thermoplastic, displaying plasticity through a range from about 37 to 40° F. to about 113° F., and showing good keeping qualities when exposed to ordinary moist atmosphere, the putty containing from 45 to 65% of carbohydrate gum, and from 6 to 25% of the amide.

2. A putty suitable for planographic printing comprising a color capable of being directly fixed on cellulose without mordanting, a corn dextrin as the essential bodying ingredient and an amide of an acid included in the group consisting of carbonic, thiocarbonic acid and cyanuric acid, all of the ionizable hydrogen atoms of the acid being amidified and the amide having at least one free reactive hydrogen atom and being present in the form of a reaction product with the dextrin, the putty being hard at room temperature, thermoplastic, displaying plasticity through a range from about 37 to 40° F. to about 113° F., and showing good keeping qualities when exposed to ordinary moist atmosphere, the putty

containing from 45 to 65% of dextrin and from 6 to 25% of the amide.

3. A putty suitable for planographic printing comprising a color capable of being directly fixed on cellulose without mordanting, a carbohydrate gum as the essential bodying ingredient and urea, the urea being present as a reaction product with the carbohydrate gum, the putty being hard at room temperature, thermoplastic, displaying plasticity through a range from about 37 to 40° F. to about 113° F., and showing good keeping qualities when exposed to ordinary moist atmosphere, the putty containing from 45 to 65% of carbohydrate gum, and from 6 to 25% of urea.

15 4. A putty suitable for planographic printing comprising a color capable of being directly fixed on cellulose without mordanting, a corn dextrin as the essential bodying ingredient and urea, the urea being present as a reaction product with the dextrin, the putty being hard at room temperature, thermoplastic, displaying plasticity through a range from about 37 to 40° F. to about 113° F., and showing good keeping qualities when exposed to ordinary moist atmosphere, the putty containing from 45 to 65% of dextrin, and from 6 to 25% of urea.

20 5. A putty suitable for planographic printing comprising a color capable of being directly fixed on cellulose without mordanting, a carbohydrate gum as the essential bodying ingredient and thiourea, the thiourea being present in the form of a reaction product with the carbohydrate gum, the putty being hard at room temperature, thermoplastic, displaying plasticity through a range from about 37 to 40° F. to about 113° F., and showing good keeping qualities when exposed to ordinary moist atmosphere, the putty containing from 45 to 65% of carbohydrate gum, and from 6 to 25% of thiourea.

25 6. A putty suitable for planographic printing comprising a color capable of being directly fixed on cellulose without mordanting, a corn dextrin as the essential bodying ingredient and thiourea, the thiourea being present in the form of a reaction product with the dextrin, the putty being hard at room temperature, thermoplastic, displaying plasticity through a range from about 37 to 40° F. to about 113° F., and showing good keeping qualities when exposed to ordinary moist atmosphere, the putty containing from 45 to 65% of dextrin and from 6 to 25% of thiourea.

30 7. A putty according to claim 1 which contains in addition a waxy material.

8. A putty according to claim 2 which contains in addition a waxy material.

35 9. A putty according to claim 1 which contains in addition a polyhydric alcohol monoester of a higher fatty acid.

10. A putty according to claim 2 which contains in addition a polyhydric alcohol monoester of a higher fatty acid.

40 11. A putty according to claim 3 which contains in addition a polyhydric alcohol monoester of a higher fatty acid.

12. A putty according to claim 4 which contains in addition a polyhydric alcohol monoester of a higher fatty acid.

45 13. A putty according to claim 5 which contains in addition a polyhydric alcohol monoester of a higher fatty acid.

14. A putty according to claim 6 which contains in addition a polyhydric alcohol monoester of a higher fatty acid.

50 15. A putty according to claim 3 which contains

in addition a soap and a polyhydric alcohol mono-ester of a higher fatty acid.

16. A putty according to claim 4 which contains in addition a soap and a polyhydric alcohol mono-ester of a higher fatty acid.

17. A putty according to claim 1 which contains in addition bentonite.

18. A putty according to claim 3 which contains in addition bentonite.

19. A putty according to claim 1 which contains a wetting agent.

5 20. A putty according to claim 3 which contains a wetting agent.

CHESTER A. AMICK.